

## UNITED STATES PATENT OFFICE.

WILLIAM MENDEL, OF BEVERLY, NEW JERSEY, ASSIGNOR TO SAMUEL A. NEIDICH,  
OF EDGEWATER PARK, NEW JERSEY.

## MANUFACTURE OF FILAMENTS AND FILMS FROM VISCOSE.

No Drawing.

Application filed May 9, 1925. Serial No. 29,228.

My invention is of particular advantage in the manufacture of filaments by projecting viscose (cellulose sulphocarbonate) through orifices into baths containing chemicals which coagulate the viscose as a semi-solid impure cellulose hydrate of sufficient strength to be handled, and an object and effect of this invention is to eliminate the impurities from such coagulated cellulose hydrate and thus improve the luster, strength and elasticity of the finished filaments.

Such coagulating or precipitating baths heretofore employed are of various kinds. For instance, because of their prompt action and relatively low cost strong acid baths, such as an aqueous solution containing eight per cent of sulphuric acid or five per cent of hydrochloric acid are commonly used for individually thin filaments such as are used in the production of artificial silk. With baths of that character, substantially all of the sulphur primarily chemically combined with the cellulose in viscose is released as free sulphur but is occluded in the mass of cellulose hydrate and impairs every desirable quality of the finished product; it being impossible to more than partially remove sulphur and its derivatives from the cellulose hydrate by the ordinary processes. Consequently, filaments thus formed have a dull yellow white surface and are comparatively weak and brittle. Organic acids and inorganic acid salts in aqueous solution have been heretofore used in such baths for lessening the aforesaid deleterious effects of sulphur and its derivatives, and with the effect that the effects of free sulphur are somewhat less apparent, but the increased cost of such additional chemicals and treatment is not economical because processes for cleansing the filaments are yet required, as in the case of the stronger acids.

I have discovered that if any suitable coagulating bath is made to include the  $\text{PO}_4$  ion, filaments of cellulose hydrate formed in such bath are practically self-cleansing because the sulphur derivatives are thereby rendered soluble in the bath; so that all of the disadvantages of the usual presence of sulphur and its derivatives, such as insoluble sulphides, are thus automatically eliminated. Such ions may be added to or produced in such baths in any convenient form or manner. However, tri-sodium phosphate

( $\text{Na}_3\text{PO}_4$ ) is a cheap vehicle for such ions and may be used in aqueous solution.

Although an aqueous solution of either mono-sodium phosphate or di-sodium phosphate or said tri-sodium phosphate alone will effect coagulation of viscose projected therein, particularly if the viscose is of low alkalinity and such solution be hot; even a small percentage, approximating a mere trace of the ion  $\text{PO}_4$  is sufficient in association or conjunction with any other suitable coagulating material. For instance, an aqueous bath containing ten per cent of sulphuric acid ( $\text{H}_2\text{SO}_4$ ) and containing ten per cent of sodium sulphate ( $\text{Na}_2\text{SO}_4$ ) is an ordinary coagulating bath which is subject to the objections aforesaid, but I find that the addition of even a fraction of one per cent of  $\text{PO}_4$  to such bath has the advantageous results above contemplated in the elimination of or prevention of formation of, insoluble sulphur derivatives in or upon the cellulose products.

Filaments thus coagulated in accordance with my invention may require no subsequent treatment other than rinsing with water and, when so treated and dried, preferably under tension, have unusually high luster, strength and elasticity.

Therefore I do not desire to limit myself to the precise details of construction, arrangement or procedure herein set forth, as it is obvious that various modifications may be made therein without departing from the essential features of my invention, as defined in the appended claims.

I claim:

1. The method of manufacturing articles from viscose which consists in coagulating viscose in an aqueous solution in which tri-sodium phosphate ( $\text{Na}_3\text{PO}_4$ ) has been dissolved with another solute capable of affecting such coagulation.

2. The method of manufacturing articles from viscose which consists in coagulating viscose in an aqueous solution in which tri-sodium phosphate ( $\text{Na}_3\text{PO}_4$ ) has been dissolved, with an acid salt solute capable of affecting such coagulation.

3. The method of manufacturing articles from viscose which consists in coagulating viscose in an aqueous solution in which tri-sodium phosphate ( $\text{Na}_3\text{PO}_4$ ) has been dissolved, with an acid solute capable of affecting such coagulation.

4. In the manufacture of cellulose articles from viscose (sulphocarbonate), the introduction of the latter into an aqueous solution resultant from mixture of water with an inorganic acid and tri-sodium phosphate.
5. In the manufacture of cellulose articles from viscose (sulphocarbonate), the introduction of the latter into an aqueous solution resultant from mixture of water with a strong mineral acid and  $\text{Na}_3\text{PO}_4$ .
6. The method of manufacturing articles from viscose which consists in coagulating viscose in an aqueous solution comprising  $\text{Na}_3\text{PO}_4$ .
7. The method of forming from cellulose sulphocarbonate a semi-solid composition which is principally cellulose hydrate, and free from deleterious sulphur compounds; which consists in coagulating liquid sulphocarbonate in an aqueous solution including an efficient acid coagulating agent, and  $\text{PO}_4$  ions in such relation with sodium phosphate as to extract such compounds from the sulphocarbonate into said aqueous solution and prevent precipitation of such compounds, 25 by holding them in said solution, independently of said cellulose hydrate.
8. The method of preventing formation of insoluble sulphur compounds during the coagulation of cellulose sulphocarbonate; 30 which consists in precipitating liquid cellulose sulphocarbonate as a semi-solid composition which is principally cellulose hydrate, and free from deleterious sulphur compounds, in an aqueous solution including an 35 efficient coagulating agent, and  $\text{PO}_4$  ions in such relation with a sodium derivative as to extract such sulphur compounds from the sulphocarbonatae into said aqueous solution and prevent precipitation of such compounds by holding them in said solution, 40 independently of said precipitated cellulose hydrate.

In testimony whereof, I have hereunto signed my name at Philadelphia, Pennsylvania, this eighth day of May, 1925. 45

WILLIAM MENDEL.